# EUROPEAN PATENT SPECIFICATION

(11) **EP 3 090 075 B1**
(45) Date of publication and mention of the grant of the patent: **05.12.2018**
(21) Application number: 14874522.7
(22) Date of filing: 28.10.2014
(51) Int. Cl.: C23C 28/02, C25D 5/14

(54) **HOT CORROSION-PROTECTED ARTICLE AND MANUFACTURE METHOD THEREFOR**
HEISSKORROSIONSGESCHÜTZTER ARTIKEL UND DESSEN HERSTELLUNGSVERFAHREN
ARTICLE PROTÉGÉ CONTRE LA CORROSION À CHAUD ET PROCÉDÉ DE FABRICATION

(30) Priority: 24.12.2013 US 201361920546 P
(43) Date of publication of application: 09.11.2016
(73) Proprietor: United Technologies Corporation, Farmington, CT 06032 (US)
(72) Inventor: TASK, Michael, N., Vernon, CT 06066 (US)
(74) Representative: Dehns
(86) International application number: PCT/US2014/062554
(87) International publication number: WO 2015/099880

(56) References cited:
- EP-A2- 1 930 467
- WO-A1-2013/037391
- US-A- 3 625 039
- US-A1- 2005 067 273
- US-A1- 2005 118 453
- US-A1- 2008 124 542
- US-A1- 2008 308 425
- US-B1- 7 364 801
- George A. Di Bari: "Electrodeposition of Nickel" In: "modern electroplating : fifth edition", 4 October 2010 (2010-10-04), john wiley, XP055223028, ISBN: 978-0-47-016778-6 pages 79-114, DOI: 10.1002/9780470602638.ch3, * Chapters 3.3-3.4 *

## Description

### BACKGROUND

The disclosure relates to gas turbines. More particularly, the disclosure relates to protective coatings for hot section components.

An exemplary gas turbine is discussed in the context of a gas turbine engine used for aircraft propulsion. Such an engine has a core gaspath passing sequentially through one or more compressor sections for compressing ingested air, a combustor section for combusting the compressed air and an introduced fuel to generate high pressure/temperature combustion gases, and one or more turbine sections for extracting work from the combustion gases to drive the compressor sections. With an exemplary turbofan engine, the turbine sections also drive a fan which, in turn drives air along a flowpath bypassing the core flowpath. Exemplary turbine sections are axial turbines wherein flow passes through one or more stages of rotating blades interspersed with stationary vanes or counter-rotating blades. The blades of a given stage may be unitarily formed with or mounted to the periphery of a disk. The disks of each section may be mounted to co-rotate with each other and any compressor section driven thereby. Exemplary compressor sections are also axial, although centrifugal compressors and turbines are also known.

Engine components (e.g., combustor panels, vanes, blades, disks, air seals, and the like) exposed to the combustion gases and heat are particularly subject to corrosion and erosion. Additionally, due to temperature increase with sequential stages of compression, the higher pressure portions of the compressor sections may be subject to significant operational heating.

A variety of substrate materials and protective coatings have been developed for these components. Exemplary substrate materials include a number of cast or powdermetallurgical (PM) forged nickel-based superalloys and/or cobalt-based superalloys. The centrifugal loading to which disks are exposed makes disks a particular area of concern for substrate materials.

US Patent 6,521,175 of Mourer, et al., issued February 18, 2003, and entitled "Superalloy optimized for high-temperature performance in high-pressure turbine disks" discloses an advanced nickel-base superalloy for powder metallurgical (PM) manufacture of turbine disks. More recent alloys have been proposed in US Patent 8,147,749, of Reynolds, issued April 3, 2012, and entitled "Superalloy compositions, articles, and methods of manufacture" and US Patent Application Publications 2013/0209265A1 and 2013/0209266A1, both of Reynolds, et al., published August 15, 2013 and entitled "Superalloy Compositions, Articles, and Methods of Manufacture".

Thermal barrier coating (TBC) systems have been developed for hot section components. Typical such systems have one or more insulative ceramic layers (e.g., zirconia-based such as yttria-stabilized zirconia (YSZ) and/or gadolinia-stabilized zirconia (GSZ)). Such coatings may be used in combination with metallic bondcoats.

On disks and certain areas of certain other components, it may be impractical or unnecessary to apply a ceramic TBC. For example, at disk rims and portions inboard thereof temperatures may be sufficiently lower than directly in the gaspath (e.g., to which airfoils are exposed) that the insulative benefit of ceramic TBC may be traded for improved hot corrosion protection of a metallic coating system.

As gas turbine operating temperatures new engine designs continue to increase relative to their predecessors, high pressure compressor disks and high pressure turbine disks are entering into a temperature regime where deposit-induced hot corrosion (even in the absence of direct exposure to combustion gas) presents a substantial durability risk. While these components (or at least some relevant portions thereof) are not exposed to combustion gas (e.g., are not directly along the core gaspath and may be partially isolated therefrom by seals and the like), deposits can develop as a result of ingestion of particulate matter from the atmosphere. In addition, substantial concentrations of SO₂ gas, which is known to exacerbate hot corrosion attack, can be present in the atmosphere in certain regions of the world. Hot corrosion is most severe in geographic regions which have elevated levels of airborne particulate matter and gaseous pollution, man-made or otherwise.

There are also substantial problems when aircraft operate in coastal regions, because ingested sea salt can also result in severe hot corrosion attack. The polycrystalline Ni-base superalloys of typical turbine and compressor disks do not have sufficient hot corrosion resistance. Thus there is an increasing need for disks (and certain legacy components) to have hot corrosion-resistant coatings in order to meet life requirements. In addition to providing hot corrosion resistance, these coatings are advantageously designed such that debits to low cycle fatigue are minimal. This can be accomplished by developing coatings that are either ductile or only loosely adherent to the superalloy substrate.

US Patent 4,346,137, of Hecht, issued August 24, 1982, and entitled "High temperature fatigue oxidation resistant coating on superalloy substrate" discloses an MCrAlY TBC bondcoat which may be used as underplatform blade coating without.

US Patent Application Publication 2010/0009092 A1, of Tryon et al., published January 14, 2010 and entitled "Economic Oxidation and Fatigue Resistant Metallic Coating" discloses another MCrAlY TBC bondcoat.

US Patent 8,124,246, of Tolpygo, issued February 28, 2012, and entitled "Coated Components and Methods of Fabricating Coated Components and Coated Turbine Disks" discloses use of sequential diffusion coating of chromium and noble metal on such a superalloy disk.

EP 1930467 describes an environmental coating suitable for use on turbine components such as turbine disks and turbine seal elements, formed of alloys susceptible to oxidation and hot corrosion.

US 2005/058848 describes a zinc-diffused nickel alloy coating for corrosion and heat protection and to a method for forming such a coating.

### SUMMARY

One aspect of the disclosure involves a coated article comprising a nickel-based superalloy substrate and a coating system atop the substrate. The coating system has a nickel-based first layer and a chromium-based second layer atop the first layer, wherein the first layer is essentially pure nickel and the second layer is essentially pure chromium.

A further embodiment may additionally and/or alternatively include the substrate being a powder metallurgical substrate.

A further embodiment may additionally and/or alternatively include the coated article being a turbine engine disk.

A further embodiment may additionally and/or alternatively include the first layer having a characteristic thickness T₁ of 13 micrometers to 51 micrometers and the second layer having a characteristic thickness T₂ of 13 micrometers to 51 micrometers.

A further embodiment may additionally and/or alternatively include the coating system consisting of said first layer and said second layer.

A further embodiment may additionally and/or alternatively include the coating system lacking a ceramic layer.

A further embodiment includes a method for manufacturing the coated article comprising a nickel-based superalloy substrate; and a coating system atop the substrate and comprising a nickel-based first layer; and a chromium-based second layer atop the first layer. The method comprises: plating the first layer; and electroplating the second layer, wherein the plating of the first layer is plating of nickel; and electroplating of the second layer is electroplating of chromium.

A further embodiment may additionally and/or alternatively include the first layer plating being electroplating.

A further embodiment may additionally and/or alternatively include forming the substrate by forging of a powder metallurgical material.

A further embodiment includes a method for using the coated article. The method comprises: installing the article in a gas turbine engine; and running the gas turbine engine to heat the article.

The details of one or more embodiments are set forth in the accompanying drawings and the description below. Other features, objects, and advantages will be apparent from the description and drawings, and from the claims.

### BRIEF DESCRIPTION OF THE DRAWINGS

FIG. 1 is an exploded partial view of a gas turbine engine turbine disk assembly.
FIG. 2 is a schematic sectional view of a surface region of the disk showing a substrate and coating.
FIG. 3 is a photomicrograph of a section of the substrate and coating.
FIG. 4 is a photomicrograph of a section of a substrate and a prior art MCrAlY overlay coating.

Like reference numbers and designations in the various drawings indicate like elements.

### DETAILED DESCRIPTION

FIG. 1 shows a gas turbine engine disk assembly 20 including a disk 22 and a plurality of blades 24. The disk is generally annular, extending from an inboard bore or hub 26 at a central aperture to an outboard rim 28. A relatively thin web 30 is radially between the bore 26 and rim 28. The periphery of the rim 28 has a circumferential array of engagement features 32 (e.g., dovetail slots) for engaging complementary features 34 of the blades 24. In other embodiments, the disk and blades may be a unitary structure (e.g., so-called "integrally bladed" rotors or disks).

The disk 22 may be formed by a powder metallurgical forging process (e.g., as is disclosed in U.S. Pat. No. 6,521,175). In an exemplary process, the elemental components of the alloy are mixed (e.g., as individual components of refined purity or alloys thereof). The mixture is melted sufficiently to eliminate component segregation. The melted mixture is atomized to form droplets of molten metal. The atomized droplets are cooled to solidify into powder particles. The powder may be screened to restrict the ranges of powder particle sizes allowed. The powder is put into a container. The container of powder is consolidated in a multi-step process involving compression and heating. The resulting consolidated powder then has essentially the full density of the alloy without the chemical segregation typical of larger castings. A blank of the consolidated powder may be forged at appropriate temperatures and deformation constraints to provide a forging with the basic disk profile. The forging is then heat treated in a multi-step process involving high temperature heating followed by a rapid cooling process or quench. The quench for the heat treatment may also form strengthening precipitates (e.g., gamma prime and eta phases) of a desired distribution of sizes and desired volume percentages. Subsequent heat treatments are used to modify these distributions to produce the requisite mechanical properties of the manufactured forging. The increased grain size is associated with good high-temperature creep-resistance and decreased rate of crack growth during the service of the manufactured forging. The heat treated forging is then subject to machining of the final profile and the slots.

FIG. 2 schematically shows a section of the disk (e.g., along a rim portion such as an outer diameter (OD) surface or a front surface or a rear surface). The disk has a forged PM substrate 100 as discussed above. A coating system 102 lies atop the substrate and has an overall thickness T. The exemplary coating system comprises a lower or inner/inboard first layer 104 (e.g., atop a surface 106 of the substrate) and an upper or outer/outboard second layer 108 (e.g., atop a surface 110 of the first layer). The respective first and second layers have thicknesses T₁ and T₂. An exemplary surface 112 of the second layer is exposed and, thus, it does not bear any further coating layer (namely, a ceramic TBC).

Exemplary T₁ is 6.0 micrometers to 50 micrometers, more narrowly 6.0 micrometers to 25 micrometers or 6.0 micrometers to 15.0 micrometers. Exemplary T₂ is 6.0 micrometers to 50 micrometers, more narrowly 6.0 micrometers to 25 micrometers or 10.0 micrometers to 20.0 micrometers.

In operation, the second layer provides corrosion resistance. The second layer consists essentially of chromium (e.g., offering equivalent performance to pure chromium). With a second layer material that is relatively brittle, the first layer provides a relatively ductile interface with the substrate to prevent cracks in the second layer from propagating into the substrate. The first layer consists essentially of nickel (e.g., offering equivalent performance to pure nickel). As applied, one or both layers may be pure or relatively pure chromium and nickel, respectively but may be subject to some diffusion with each other or the substrate.

An exemplary process for depositing the first layer is plating (e.g., electroless or electroplating). This may be applied directly to the machined substrate to build to the thickness T₁.

The second layer is deposited by electroplating. This is applied directly to the first layer (e.g., after any washing) to build to the thickness T₂. Exemplary electroplating is disclosed in US Patent Application Publication 2013/0220819 entitled "Electrodeposition of Chromium from Trivalent Chromium Using Modulated Electric Fields". Such use of a trivalent chromium bath avoids toxicity concerns of hexavalent chromium.

FIG. 3 is a micrograph of an exemplary such two layer coating system 102. The lower layer 104 is directly atop the substrate and is thinner than the upper layer 104 (e.g. about 15% to 33% of the upper layer thickness). For comparison, FIG. 4 shows a baseline MCrAlY. Several things appear. First, it is seen that cracks 120 in the upper layer 108 normal to the surface (outer surfaces 106, 110, and 112 of the substrate and respective layers) have not propagated into the lower layer 104. The lower layer ductility, is believed to help avoid such crack propagation. In operation, these cracks 120 may effectively seal up with a protective Cr₂O₃ scale during exposure which may add to robustness and protection.

Second, a dark boundary 122 is seen between the two layers. This is a very thin gap that appears to have been created during the sectioning/mounting process for generating the micrograph. Also, it is seen that, compared to the MCrAlY, there is a lower degree of apparent interdiffusion with the substrate. Finally, it is seen that, compared to the MCrAlY, there is a lower degree of apparent surface roughness of the exposed coating surface.

## Claims

1. A coated article (22) comprising:
a nickel-based superalloy substrate (100); and
a coating system (102) atop the substrate and comprising:
a nickel-based first layer (104); and
a chromium-based second layer (108) atop the first layer, wherein:
the first layer is essentially pure nickel; and
the second layer is essentially pure chromium.

2. The coated article of claim 1 wherein:
the substrate is a powder metallurgical substrate.

3. The coated article of claim 1 or claim 2 being a turbine engine disk.

4. The coated article of any preceding claim wherein:
the first layer has a characteristic thickness T₁ of 13 micrometers to 51 micrometers; and
the second layer has a characteristic thickness T₂ of 13 micrometers to 51 micrometers.

5. The coated article of any preceding claim wherein:
the coating system consists of said first layer and said second layer.

6. The coated article of any one of claims 1-4 wherein:
the coating system lacks a ceramic layer.

7. A method for using the coated article of any of claims 1-6, the method comprising:
installing the article in a gas turbine engine; and
running the gas turbine engine to heat the article.

8. A method for manufacturing a coated article comprising:
a nickel-based superalloy substrate (100); and
a coating system (102) atop the substrate and comprising:
a nickel-based first layer (104); and
a chromium-based second layer (108) atop the first layer, the method comprising:
plating the first layer; and
electroplating the second layer,
wherein the plating of the first layer is plating of nickel;
and the electroplating of the second layer is electroplating of chromium.

9. The method of claim 8 wherein:
the first layer plating is electroplating.

10. The method of claim 8 or claim 9, further comprising:
forming the substrate by forging of a powder metallurgical material.

11. The method of any of claims 8-10 wherein:
the first layer has a characteristic thickness of 13 micrometers to 51 micrometers; and
the second layer has a characteristic thickness of 13 micrometers to 51 micrometers.

12. The method of any of claims 8-11 wherein:
the coating system consists of said first layer and said second layer.

13. The method of any of claims 8-11 wherein the coating system of the coated article lacks a ceramic layer.

14. The method of any of claims 8-13 wherein the coated article is a turbine engine disk.

## Patentansprüche

1. Beschichteter Artikel (22), umfassend:
ein Superlegierungs-Substrat auf Nickelbasis (100); und
ein Beschichtungssystem (102) auf dem Substrat und umfassend:
eine erste Schicht auf Nickelbasis (104); und
eine zweite Schicht auf Chrombasis (108) auf der ersten Schicht,
wobei:
die erste Schicht im Wesentlichen reines Nickel ist; und
die zweite Schicht im Wesentlichen reines Chrom ist.

2. Beschichteter Artikel nach Anspruch 1, wobei:
das Substrat ein pulvermetallurgisches Substrat ist.

3. Beschichteter Artikel nach Anspruch 1 oder Anspruch 2, wobei dieser eine Turbinentriebwerkscheibe ist.

4. Beschichteter Artikel nach einem der vorstehenden Ansprüche, wobei:
die erste Schicht eine charakteristische Dicke T₁ von 13 Mikrometer bis 51 Mikrometer aufweist; und
die zweite Schicht eine charakteristische Dicke T₂ von 13 Mikrometer bis 51 Mikrometer aufweist.

5. Beschichteter Artikel nach einem der vorstehenden Ansprüche, wobei:
das Beschichtungssystem aus der ersten Schicht und der zweiten Schicht besteht.

6. Beschichteter Artikel nach einem der Ansprüche 1 - 4, wobei:
das Beschichtungssystem keine keramische Schicht aufweist.

7. Verfahren zur Verwendung des beschichteten Artikels nach einem der Ansprüche 1 - 6, wobei das Verfahren Folgendes umfasst:
Einbauen des Artikels in ein Gasturbinentriebwerk; und
Laufenlassen des Gasturbinentriebwerks, um den Artikel zu erhitzen.

8. Verfahren zur Herstellung eines beschichteten Artikels, umfassend:
ein Superlegierungssubstrat auf Nickelbasis (100); und
ein Beschichtungssystem (102) auf dem Substrat und umfassend:
eine erste Schicht auf Nickelbasis (104); und
eine zweite Schicht auf Chrombasis (108) auf der ersten Schicht,
wobei das Verfahren Folgendes umfasst:
Plattieren der ersten Schicht; und
Elektroplattieren der zweiten Schicht,
wobei das Plattieren der ersten Schicht das Plattieren von Nickel ist;
und wobei das Elektroplattieren der zweiten Schicht das Elektroplattieren von Chrom ist.

9. Verfahren nach Anspruch 8, wobei:
das Plattieren der ersten Schicht Elektroplattieren ist.

10. Verfahren nach Anspruch 8 oder Anspruch 9, weiter umfassend:
Bilden des Substrats durch Schmieden eines pulvermetallurgischen Materials.

11. Verfahren nach einem der Ansprüche 8 - 10, wobei:
die erste Schicht eine charakteristische Dicke von 13 Mikrometer bis 51 Mikrometer aufweist; und
die zweite Schicht eine charakteristische Dicke von 13 Mikrometer bis 51 Mikrometer aufweist.

12. Verfahren nach einem der Ansprüche 8 - 11, wobei:
das Beschichtungssystem aus der ersten Schicht und der zweiten Schicht besteht.

13. Verfahren nach einem der Ansprüche 8 - 11, wobei das Beschichtungssystem des beschichteten Artikels keine keramische Schicht aufweist.

14. Verfahren nach einem der Ansprüche 8 - 13, wobei der beschichtete Artikel eine Turbinentriebwerkscheibe ist.

## Revendications

1. Article revêtu (22) comprenant :
un substrat en superalliage à base de nickel (100) ; et
un système de revêtement (102) au-dessus du substrat et comprenant :
une première couche à base de nickel (104) ; et
une seconde couche à base de chrome (108) au-dessus de la première couche,
dans lequel :
la première couche est du nickel essentiellement pur ; et
la seconde couche est du chrome essentiellement pur.

2. Article revêtu selon la revendication 1, dans lequel :
le substrat est un substrat métallurgique en poudre.

3. Article revêtu selon la revendication 1 ou la revendication 2, qui est un disque de moteur à turbine.

4. Article revêtu selon l'une quelconque des revendications précédentes, dans lequel :
la première couche a une épaisseur caractéristique T₁ de 13 micromètres à 51 micromètres ; et
la seconde couche a une épaisseur caractéristique T₂ de 13 micromètres à 51 micromètres.

5. Article revêtu selon l'une quelconque des revendications précédentes, dans lequel :
le système de revêtement se compose de ladite première couche et de ladite seconde couche.

6. Article revêtu selon l'une quelconque des revendications 1 à 4, dans lequel :
le système de revêtement est dépourvu de couche céramique.

7. Procédé pour utiliser l'article revêtu selon l'une quelconque des revendications 1 à 6, le procédé comprenant :
l'installation de l'article dans un moteur à turbine à gaz ; et
la mise en fonctionnement du moteur à turbine à gaz pour chauffer l'article.

8. Procédé de fabrication d'un article revêtu comprenant :
un substrat en superalliage à base de nickel (100) ; et
un système de revêtement (102) au-dessus du substrat et comprenant :
une première couche à base de nickel (104) ; et
une seconde couche à base de chrome (108) au-dessus de la première couche, le procédé comprenant :
le dépôt de la première couche ; et
l'électrodéposition de la seconde couche,
dans lequel le dépôt de la première couche est un nickelage ;
et l'électrodéposition de la seconde couche est une électrodéposition de chrome.

9. Procédé selon la revendication 8, dans lequel :
le dépôt de la première couche est une électrodéposition.

10. Procédé selon la revendication 8 ou la revendication 9, comprenant en outre :
la formation du substrat par forgeage d'un matériau métallurgique en poudre.

11. Procédé selon l'une quelconque des revendications 8 à 10, dans lequel :
la première couche a une épaisseur caractéristique de 13 micromètres à 51 micromètres ; et
la seconde couche a une épaisseur caractéristique de 13 micromètres à 51 micromètres.

12. Procédé selon l'une quelconque des revendications 8 à 11, dans lequel :
le système de revêtement se compose de ladite première couche et de ladite seconde couche.

13. Procédé selon l'une quelconque des revendications 8 à 11, dans lequel le système de revêtement de l'article revêtu est dépourvu de couche céramique.

14. Procédé selon l'une quelconque des revendications 8 à 13, dans lequel l'article revêtu est un disque de moteur à turbine.
